

## UNITED STATES PATENT OFFICE.

HENRY NOEL POTTER, OF GÖTTINGEN, GERMANY, ASSIGNOR TO GEORGE WESTINGHOUSE, OF PITTSBURG, PENNSYLVANIA.

## INSULATING COMPOUND.

SPECIFICATION forming part of Letters Patent No. 694,989, dated March 11, 1902.

Application filed August 9, 1899. Serial No. 726,622. (No specimens.)

107-58

To all whom it may concern:

Be it known that I, HENRY NOEL POTTER, a citizen of the United States of America, and a resident of Göttingen, Germany, have invented certain new and useful Improvements in Insulating Compounds, of which the following is a specification.

I have devised a new insulating compound, which I have used in my recent electrical work, and I find it admirably suited to the purpose of an electrical insulator, possessing qualities which particularly adapt it to be conveniently manufactured in the form of small insulating bodies for carrying circuit-  
10 terminals and keeping them insulated from each other. One quality of this material which especially adapts it for the purpose last mentioned is that large numbers of pieces formed from it can be packed together and  
15 baked without danger of their becoming fixed together. In this respect and also in its ability to resist heat the material is superior to porcelain, while its insulating qualities are sufficiently high for ordinary electrical uses.  
20 The material which I have devised consists, mainly, of soapstone or talc-powder mixed with water and some binder, such as tragacanth, dextrose, or the like. The proportions in which I usually mix the elements men-  
25 tioned are: one hundred parts soapstone or talc-powder, fifteen parts tragacanth, and thirty-five to forty-five parts water. These elements are first mixed to form a paste or dough and are then molded or otherwise  
30 formed into the desired shapes, after which they are dried, and when the drying process is complete they are either baked separately or packed together and subjected to the baking process. I find that they can safely be  
35 packed in this way and that there is little or no tendency for the pieces becoming attached to each other during the baking.

The insulating compound above described is well adapted after its final treatment to resist the effects of intense heat. The compound is exceedingly light in weight and possesses the advantage due to such lightness.

I may add to the described mixture from two to four parts of magnesium chlorid or a magnesium nitrate. Should the insulating material be designed for use in places where there is little or no danger of exposure to great heat, I sometimes add to the mixture first described about five to fifteen per cent. of water-glass. This addition has the effect of making the compound much harder and mechanically considerably stronger. For many uses the compound containing water-glass would be preferable to one which lacked that element. I have given to the compound, whether containing the water-glass or not, the name "talcite," and I desire in the present application to claim this compound as a means of electrical insulation, it being understood that for special purposes I may employ slightly-  
55 varying proportions of the elements named.

I claim as my invention—

1. A highly-refractory electrical insulating material, consisting of soapstone or talc-powder and water combined with a binder such as tragacanth, the soapstone or talc-powder being largely in excess of the other materials.

2. A highly-refractory electrical insulating material, consisting of soapstone or talc-powder, water, a binding material such as tragacanth and admixture of water-glass, the soapstone or talc-powder being largely in excess of the other materials.

Signed by me at Hanover, Germany, this 14th day of July, 1899.

HENRY NOEL POTTER.

Witnesses:

W. K. ANDERSON,  
KIRKE LATHROP.